

June 6, 1939.

W. HIRSCHKIND ET AL

2,161,045

BLEACHING

Original Filed June 1, 1937 6 Sheets-Sheet 1



FIG. 1

FIG. 2



FIG. 3



BY

INVENTORS  
Wilhelm Hirschkind  
Earl G. Thompson  
David J. Pye  
Robert H. Eckhoff  
ATTORNEY

June 6, 1939.

W. HIRSCHKIND ET AL.

2,161,045

BLEACHING

Original Filed June 1, 1937

6 Sheets-Sheet 2



INVENTORS  
Wilhelm Hirschkind  
Earl G. Thompson  
David J. Pye  
BY  
Robert H. Eckhoff  
ATTORNEY

June 6, 1939.

W. HIRSCHKIND ET AL

2,161,045

BLEACHING

Original Filed June 1, 1937 6 Sheets-Sheet 3

FIG. 5



BY

INVENTORS  
Wilhelm Hirschkind  
Earl G. Thompson  
David J. Pye  
Robert H. Eckhoff.  
ATTORNEY.

June 6, 1939.

W. HIRSCHKIND ET AL

2,161,045

BLEACHING

Original Filed June 1, 1937

6 Sheets-Sheet 4

FIG. 6



INVENTORS  
Wilhelm Hirschkind  
Earl G. Thompson  
David J. Pye  
BY  
Robert H. Eckhoff  
ATTORNEY.

June 6, 1939.

W. HIRSCHKIND ET AL

2,161,045

BLEACHING

Original Filed June 1, 1937

6 Sheets-Sheet 5



FIG-7-



FIG-8-

INVENTORS  
Wilhelm Hirschkind  
Earl G. Thompson  
David J. Pye  
BY  
Robert H. Eckloff  
ATTORNEY.

June 6, 1939.

W. HIRSCHKIND ET AL

2,161,045

BLEACHING

Original Filed June 1, 1937 6 Sheets-Sheet 6



FIG. 9

INVENTORS  
Wilhelm Hirschkind  
Earl G. Thompson  
David J. Dye  
BY  
Robert H. Eckhoff  
ATTORNEY.

Patented June 6, 1939

2,161,045

# UNITED STATES PATENT OFFICE

2,161,045

## BLEACHING

Wilhelm Hirschkind, Berkeley, David J. Pye, Pittsburgh, Calif., and Earl G. Thompson, Seattle, Wash., assignors, by mesne assignments, to The Dow Chemical Company, Midland, Mich., a corporation of Michigan

Application June 1, 1937, Serial No. 145,806  
Renewed November 7, 1938

### 12 Claims.

(Cl. 8—106)

This invention relates to improvements in the use of oxidizing materials, particularly materials which are used to effect oxidizing bleaches. Such materials include chlorine, hypochlorous acid, the 5 hypochlorites, water solutions of chlorine, hydrogen peroxide, peroxides, and per salts as perborates, persulphates, and permanganates. The invention is broadly applicable to the bleaching of materials generally, but it will be described in 10 connection with the bleaching of cellulose materials, particularly wood pulps such as sulphite, soda and kraft pulps. However, it is to be understood that this is only disclosed as a typical application of the invention which is also useful on 15 other materials as well as pulps, for example, to the bleaching of cloths, rags, wool and other materials.

Cellulose pulps are ordinarily bleached with chlorine water, hypochlorous acid, or hypochlorites. The initial portion of the bleaching treatment, whether the treatment be conducted in a single or a plurality of stages, if analyzed, will be found to be a chlorination step. That is, materials in the pulp are chlorinated by the available chlorine or by the hypochlorite to form chlorinated addition and substitution products. Further treatment of the pulp is thereafter conducted to oxidize coloring material. Between the chlorination and oxidizing treatment, the pulp 30 may or may not be washed to remove the soluble chlorinated materials with acid, alkaline or plain water washes.

The action of light upon the bleaching of cellulose has previously been studied by various investigators, including Escourrou. He reported (Congres de la Papeterie, June, 1928, and Chimie et Industrie, June, 1928) that while the ultra violet light sensibly diminished the time of bleaching, it resulted in a greater consumption of chlorine and, 40 because the chlorine became more active, a cellulose attack occurred which lowered the yield. Further, Escourrou found that the bleached cellulose was rich in oxy and hydroxy celluloses, the presence of which was revealed by an appreciable 45 elevation in the copper number. Escourrou reported an undesirable decrease in the alpha cellulose content and an increase in the formation of beta and gamma celluloses. These findings led him to advise against the use of light bleaching, 50 particularly if the pulp was destined for the manufacture of viscose silk.

As a result of investigations hereinafter set forth, we have arrived at the conclusion that the reason Escourrou did not find the use of light 55 advantageous was that while he used light from a quartz mercury arc, reporting that its spectrum contained a group of particularly intense rays in the neighborhood of 365 millimicrons, this light source also contains light rays of a shorter length, as low as 180 millimicrons, which Escourrou did

not eliminate. We have secured excellent results by confining the light to a wave length not substantially beyond 300 millimicrons. In fact, the broad effective band which we prefer is between 300 and 420 millimicrons. Beyond 420 millimicrons, the visible light present is not of any appreciable value. The effective light band is that passed by a boro-silicate glass such as Crown glass or Pyrex. Apparently light rays shorter than about 300 millimicrons have a detrimental 10 effect upon cellulose, and hence the reason for Escourrou's finding. The specific preferred light for use on wood pulp is that having a wave length of 365 millimicrons.

It is in general the broad object of the present 15 invention to provide a bleaching process in which light can be used effectively to improve the quality of the bleached product.

Another object of the invention is to provide an improvement in bleaching wherein a selected 20 light band is effectively used to improve the color without damage to the bleached material.

The invention includes other objects and features of advantage some of which, together with the foregoing, will appear hereinafter wherein the 25 present preferred practice is disclosed.

A further object of the invention is to improve the oxidizing ability, of oxidizing materials used for bleaching, as measured by color improvement.

In the drawings accompanying and forming a 30 part hereof Figure 1 illustrates the decomposition rate of various solutions when subject to light for the time indicated.

Figure 2 illustrates the chlorine consumption 35 rate of a pulp treated with a 3% chlorine water with and without light.

Figure 3 illustrates the relative chlorine consumption of the same pulp treated initially in the 40 dark and thereafter divided and treated with and without light.

Figures 4 and 5 illustrate the chlorine consumption, the viscosity, copper number and percent of alpha cellulose in a pulp treated with and without light. Figure 4 shows the first stage 45 treatment and Figure 5 shows the second stage treatment.

Figure 6 illustrates the same factors as in Figures 4 and 5 applied to the second stage, of another pulp.

Figures 7 and 8 indicate second stage chlorine 50 consumption values on a sulphite pulp.

Figure 9 illustrates diagrammatically the absorption characteristics of pulp and the coloring matter therein.

Referring to Figure 1, we have determined the rate of chlorine evolution from a hypochlorite solution, a hypochlorous acid solution, an 18% hydrochloric acid solution, and a solution of chlorine in water. The results, as set forth in 60

Figure 1, indicate that the light is much more effective on the hypochlorous acid than on the chlorine. It is to be noted that the sodium hypochlorite is relatively stable under the light. 5 The conclusion drawn from this is that any improved results are due to something other than an increase in the rate of decomposition of the hypochlorite.

Escourrou subjected the pulp undergoing treatment to the action of ultra violet light during the chlorination stage. We have investigated the comparative value of light during the chlorination stage and during the oxidation stage in various chlorine bleaches and we have determined 10 that the light is not particularly effective during the chlorination stage treatment of the cellulose.

Referring to Figure 2, it is to be noted that the chlorination stage is indicated by a high 20 percentage chlorine consumption in the first five minutes at the particular chlorine concentration. Thereafter, in the presence of light, the chlorine consumption proceeds at a second very definite rate, while, in case light is absent, some few 25 minutes elapse before the second rate of chlorine consumption is definitely established. There is an interval of secondary reaction which cannot be definitely explained but which is eliminated by the use of light, during the chlorination 30 operation. The value of this secondary reaction will be discussed hereinafter in connection with Figure 4.

The pulp tested in this instance (Figure 2), a sulphite pulp, was placed in a five gallon crock at 35 a 2% consistency. A 400 watt G. E. mercury vapor lamp was placed in the center of the crock and was shielded from the pulp by a suitable boro-silicate glass which eliminated substantially all light shorter than 300 millimicrons. A cooling water jacket was provided to keep the temperature of the pulp below 30° C. The annular ring of pulp surrounding the light was about 3 inches in thickness, with a minimum radius of 3 inches from the light pencil as the center.

45 We have separated the encrusting material from a cellulose pulp, making an extract or infusion thereof. This material, when subject to light, was found to selectively absorb light between 300 and 420 millimicrons. The material particularly absorbed the 365 millimicron band. This means that in subjecting material to an oxidizing bleach, one should determine the light band selectively absorbed by the material to be treated. Thereafter, this light band can 50 be used to enhance the action of the oxidizing bleaching agent, and any detrimental effects can be obviated by limiting the light to the band effectively absorbed by the material to be treated. This will be further discussed hereinafter in connection with Figure 9.

We have subjected pulp and other materials to the action of various oxidizing chemicals while irradiating with light selectively absorbed substantially only by the encrusting or color imparting material. In some cases we used light containing bands shorter than 300 millimicrons and in these instances poor results were obtained as manifested by high reagent consumption, degradation of the material treated and little color improvement. This confirmed Escourrou's findings. In other cases we restricted the light substantially to that selectively absorbed by the encrusting or coloring material and in these instances the reagent economy was increased, degradation was eliminated or at a minimum, 70 75

while material color improvement was observed. The irradiating light should be restricted to that selectively absorbed by the encrusting material, that light selectively absorbed by the other material, cellulose, for example, being substantially 5 absent.

Hereinafter we have disclosed the application of the invention to various materials and various oxidizing chemicals.

We have used light of 300 millimicrons and above effectively in treating cellulose, both in single stage and in multi stage operations. In Figure 3 is shown the chlorine consumption on a sulphite pulp in the first stage. The sample was treated with 3% of chlorine for thirty minutes. 10 This is equivalent to a chlorination operation. After this, the light was turned on and the increase in chlorine consumption is plainly indicated upon that portion of the sample which was subject to the light, as compared to that which 20 was permitted to remain merely in the original condition. The color of the pulp treated under the light was very much brighter than that run under normal conditions, that is without the use of the light during the last portion of the single 25 stage treatment.

In multi stage bleaching (Figures 4 and 5), chemical tests were made on samples taken at intervals from two bleach batches, run with light and without light. The original pulp was a 30 sulphite pulp. The first stage operation consisted of the 3% chlorine water bleach and 2% consistency for a total of sixty minutes (Figure 4). After washing, a second stage (Figure 5) of one hundred and twenty minute treatment was 35 given with 1.5% of  $\text{Cl}_2$  as hypochlorite at a 2% pulp consistency. The temperature was kept below 30° C. at all times. Viscosity, copper number and alpha cellulose values were run upon each of the pulps during the bleaching operation, during both the first and second stages. It is to be noted in Figure 4 that the viscosity of the un- 40 radiated pulp dropped to a much lower value with the increased degree of chlorination. The increase in viscosity thereafter is connected with some secondary reaction which causes the chlorine consumption rate to proceed at a practically 45 constant value between the ten and forty minute points before the reaction rate falls off to nearly zero (see Curve D, Figure 2). The secondary 50 reaction does not seem to take place in the irradiated pulp, this being indicated by the constant decrease in viscosity which signifies a substantially pure oxidation process. The copper number shown in Figure 4, indicative of the degree 55 of degradation of the pulp (approximately proportional to the reciprocal of the viscosity) does not indicate any detrimental action upon the pulp. Likewise the alpha cellulose value shown in Figure 4 indicates the selected light band does 60 not have any detrimental effect.

The second stage viscosity shown in Figure 6 shows a marked increase. This is followed by a decrease in viscosity directly correlated with the oxidation of the pulp. The slight drop in the 65 viscosity is inconsequential in view of the tremendous improvement in color.

To determine further whether or not light has any harmful effect upon the pulp, twelve liters of a 2% pulp were treated for a half hour using 70 3% chlorine in the first stage. The pulp was then washed and bleached for a half hour using 1.5% chlorine as  $\text{NaOCl}$ . After the initial half hour period, the pulp was subjected to the Pyrex glass screened light (above 300 millimicron 75

band) from a mercury vapor lamp in the apparatus previously described. The test was carried out over a prolonged period of eight hours (480 minutes). The first stage treatment corresponded to that previously disclosed except that it was discontinued after one half hour. In Figure 6 we have shown the factors indicating that the long treatment of the irradiated pulp did not harm the pulp.

Another sample of the pulp bleached in the first stage for thirty minutes was washed and then treated for ten minutes at a 3% consistency with 0.5% NaOH solution and then washed again. The second stage was then carried out by treating with 1.5% chlorine as NaOCl at a 2% consistency. The pulp was treated for thirty minutes without irradiation and then with radiation over a period of four hours. The resulting bleached pulp was of a very high order of brightness. This maximum practical brightness was reached after only two hours and was of the same brightness as the eight hour sheet of the previous two stage bleach.

The invention is applicable to the bleaching of materials generally. It can be used to advantage in any case wherein an oxidizing bleach is employed. Cellulosic materials as the aforementioned pulps are most advantageously treated. Some pieces of unbleached muslin were treated in a single stage CaOCl<sub>2</sub> bleach using 6% available chlorine. One sample was radiated directly with ultra violet light from the quartz lamp, the second was radiated with light from the same source but filtered through Pyrex glass and the third sample was treated without light as a control. The bleach was somewhat slower and the chlorine consumption in the unradiated sample was more constant than in pulp bleaching but the general effect of the light is identical with that on the wood pulp. The filtered light greatly speeds up the bleach and results in a higher color while the direct radiated bleach is inefficient from a chlorine consumption standpoint. The brightness and chlorine consumption are shown below:

| 45 | Sample                     | Bright-<br>ness | Percent Cl <sub>2</sub><br>consumed |
|----|----------------------------|-----------------|-------------------------------------|
|    | No light.....              | 84.6            | 60                                  |
|    | Direct ultra violet.....   | 81.5            | 98                                  |
|    | Filtered ultra violet..... | 85.5            | 95                                  |

The utility of other bleach materials, for example, a peroxide, has been established. In one instance, a sulphite pulp was treated in the first stage chlorination in a manner similar to that hereinbefore set forth, using 5% chlorine as the chlorinating material and following this with an alkaline wash. The second stage samples were treated with 1.0% H<sub>2</sub>O<sub>2</sub> (on the weight of pulp) after being made alkaline with calcium hydroxide. The hydrogen peroxide, in the concentration employed, was equivalent in oxidizing power to 2% available chlorine. Samples were radiated immediately upon addition of the hydrogen peroxide, one sample being radiated with a Pyrex filtered light and the other was kept in the dark in the control. The peroxide bleach was extremely slow, so the bleach was prolonged for four hours until 50% of the oxidizing power had been consumed. The samples were treated the same length of time, but the radiated samples showed a brightness of 89.3 as against 86.5 for the un-irradiated samples. The details of the apparatus and the treatment employed are given hereinafter in connection with the investigation on sulfite pulp.

That the shorter ultra violet rays cause a degradation of the cellulose in the presence of effective oxidizing agents, and that this presents the reason why Escourrou's investigation failed, is amply established by the investigation conducted by us upon sulfite pulps.

Sulfite pulp was treated in each case with a thirty minute first stage chlorine bleach at 4% consistency using 5% Cl<sub>2</sub> on the weight of stock. The bleached pulp was then washed and the soluble chlorinated lignin extracted with a 0.2% NaOH wash. The second stage bleach was run at 2.5% consistency using 1.5% Cl<sub>2</sub> as CaOCl<sub>2</sub>. The first thirty minutes of the bleach was performed without light for all tests. One sample was then treated in a crystallizing dish 4" below the direct radiation of a G. E. quartz mercury vapor lamp, the second sample was treated similarly but the light was screened through a 5 mm. sheet of Pyrex glass and the third sample was left as a control using no light. Figure 7 shows the chlorine consumption for the three samples and the brightness and copper numbers are given below.

| 25 | Sample treatment                 | Bright-<br>ness | Copper<br>number | Percent Cl <sub>2</sub><br>consumed |
|----|----------------------------------|-----------------|------------------|-------------------------------------|
|    | No light.....                    | 86.5            | 2.08             | 18.5                                |
|    | Direct ultra violet.....         | 89.0            | 2.9              | 53                                  |
|    | Pyrex filtered ultra violet..... | 90.5            | 1.8              | 43                                  |

A second test identical with the previous one was run using 3% Cl<sub>2</sub> in the second stage to induce overbleaching to a more marked degree. The chlorine consumption curves are shown in Figure 8 and the brightness, copper number, etc., are shown below.

| 35 | Sample treatment                    | Bright-<br>ness | Copper<br>number | Alpha-<br>cellulose | Percent Cl <sub>2</sub><br>consumed |
|----|-------------------------------------|-----------------|------------------|---------------------|-------------------------------------|
|    | No light.....                       | 89.5            | 1.23             | 89.2                | 11                                  |
|    | Direct ultra violet.....            | 90.5            | 2.04             | 85.5                | 72                                  |
|    | Pyrex filtered ultra<br>violet..... | 91.8            | 1.40             | 88.5                | 72                                  |

It can be seen from the comparison of the chlorine consumed in each case with the color obtained that the efficiency of the direct radiated pulp bleach is lower than that of the filtered ultra violet bleach due to the fact that the chlorine in the former bleach went partially to forming oxycellulose and was very likely decomposed directly by the short ultra violet. The term "efficiency" here used refers to the ratio of brightness increase to chlorine consumed.

Light absorption by cellulose starts somewhat below 360 millimicrons. On the other hand, the bleachable lignin or discoloring matter, the encrusting matter in pulp, starts absorbing light in the region of 420 millimicrons, and extends at least on to 300 millimicrons and perhaps farther. Apparently the longer or near ultra violet light of less energy is sufficient to activate the lignin, which is more reactive than the cellulose, but the relatively stable cellulose molecule requires the higher energy of the farther ultra violet light in order that the formation of oxycellulose may be enhanced. This has been amply established by us because we have determined that if the light band be restricted to between 300 and 420 millimicrons, and if in fact the light band is kept at the suggested 365 millimicrons for lignin containing materials of the character heretofore dealt with, then effective and improved bleaching of the pulp is readily obtained without degrading the cellulose due to the radiation of the pulp.

Upon other materials the effective light band may be found to have other limits but the determination of these is a simple matter of determining the bands selectively absorbed by the material to be oxidized and that to be unaffected. The irradiations are then restricted to that absorbed by the material to be oxidized so that it alone is activated. This is illustrated in Figure 9 wherein the absorption characteristics of the 10 coloring matter and of a bleached sulfite pulp are shown. The coloring matter absorption is indicated by line A and that of the bleached pulp by line B. To activate the coloring matter selectively while avoiding the degradation of the pulps 15 one should restrict the irradiation so that little, if any, effective radiations below line C are included. Practically, the only effective radiations for the coloring matter which are not harmful to the cellulose are those included in the shaded 20 area of Figure 9.

With other wood pulps and with other materials the relative positions of lines A and B may shift, and it may be necessary to use light having other effective wave lengths. The determination 25 and selection is a simple matter of determining the absorption of the coloring matter and the absorption of the other matter present which is not to be affected. With these measurements available one eliminates from the irradiations 30 passed to the material that light harmful to the other material. This is a simple matter of light absorption measurement readily made by one skilled in the art.

The light source utilized in some of the present 35 work was a mercury vapor General Electric lamp designated as H-1. This lamp has an inherent emission capacity for the 365 m. m. band, furnishing this radiation at comparatively high intensity. The only shorter band emitted is the 334 40 band. The intensity of this emission is low and the band is readily eliminated by a suitable filter.

Because the present invention enables bright 45 pulps to be secured, activating the oxidizable coloring material, low temperature operation is made feasible and we have successfully bleached pulps at 20°-25° C. and below. This means an increase in steam economy with even increased 50 brightness. At high temperatures the present invention enables the time of treatment to be shortened, thus avoiding pulp degradation due to heat.

Because of the desirability of uniform pulp 55 radiation low pulp density is a factor for consideration. We have successfully worked at high and low densities but we prefer about a 5% density.

Reference has heretofore been made to measurement of the light absorption characteristics 60 of the bleached pulp, as distinguished from cellulose. This has been done because after all the pulp is mainly cellulose and the two, in this sense, are synonymous. Another consideration is that in fact one does not wish to degrade the pulp and, therefore, if other components are 65 present, besides the cellulose, these are not to be activated.

The process of the present invention is applicable to oxidizing operations generally as performed on cellulose materials. It is particularly 70 useful in producing high alpha cellulose pulps.

We claim:

1. The step of improving a cellulosic material 75 undergoing an oxidizing bleach which consists in irradiating the material with only those light

waves longer than 300 millimicrons and below 420 millimicrons.

2. The step of improving a cellulosic material undergoing an oxidizing bleach with a material selected from the group consisting of chlorine, 5 hypochlorous acid and a hypochlorite, which consists in irradiating the material with only those light waves longer than 300 millimicrons and below 420 millimicrons.

3. Irradiating a cellulose material, undergoing 10 a treatment with a material selected from the group consisting of chlorine, hypochlorous acid and a hypochlorite, in the presence of water, with light filtered through a Pyrex filter.

4. In a process of improving the quality of a 15 cellulose pulp the step which includes subjecting the pulp, in aqueous suspension in the presence of a material selected from the group consisting of chlorine, hypochlorous acid and a hypochlorite, to the action of effective light all of a wavelength substantially longer than 300 millimicrons. 20

5. A process of improving the quality of a cellulose pulp which includes subjecting the pulp, in aqueous suspension, to the action of effective light all of a wavelength substantially longer than 25 300 millimicrons while said pulp is undergoing an oxidizing phase of a bleaching operation.

6. The step of improving a cellulosic material undergoing an oxidizing bleach which consists in 30 irradiating the material with light waves all substantially longer than 300 millimicrons.

7. The step of improving a cellulosic material undergoing an oxidizing bleach with a material selected from the group consisting of chlorine, 35 hypochlorous acid and a hypochlorite, which consists in irradiating the material with light waves all substantially longer than 300 millimicrons.

8. In a process of single stage bleaching of 40 an aqueous suspension of a cellulose pulp, the steps of subjecting said pulp to the action of a hypochlorite for a portion of the normal operating time in said stage and then irradiating said pulp with light waves all substantially longer 45 than 300 millimicrons.

9. In a multi-stage bleaching operation, the steps of subjecting an aqueous suspension of a 50 pulp to chlorination, and subjecting said pulp to the further action of a material selected from the group consisting of chlorine, hypochlorous acid and a hypochlorite to bleach said pulp while irradiating said pulp with light rays all substantially longer than 300 millimicrons.

10. Bleaching a wood pulp with an oxidizing 55 bleach agent while irradiating said pulp with light of 365 millimicrons as the only substantially effective irradiating light.

11. The step in improving the quality of a cellulose material which consists in irradiating said 60 material with only those light waves longer than 300 millimicrons and shorter than 420 millimicrons while subjecting said material to an oxidizing bleach with a per compound.

12. The step in improving the quality of a cellulose material which consists in irradiating said 65 material with only those light waves longer than 300 millimicrons and below 420 millimicrons while subjecting said material to an oxidizing bleach with a material selected from the group 70 consisting of a peroxide, a perborate, a persulfate, a permanganate and hydrogen peroxide.

WILHELM HIRSCHKIND.

DAVID J. PYE.

EARL G. THOMPSON.